

L. EDEL.  
METHOD OF CASTING.  
APPLICATION FILED NOV. 29, 1916.

1,224,618.

Patented May 1, 1917.



INVENTOR:

LUCAS EDEL,

KNIGHT & COOK, execs.

By

# UNITED STATES PATENT OFFICE.

LUCAS EDEL, OF ST. LOUIS, MISSOURI.

## METHOD OF CASTING.

1,224,618.

Specification of Letters Patent.

Patented May 1, 1917.

Application filed November 29, 1916. Serial No. 134,032.

To all whom it may concern:

Be it known that I, LUCAS EDEL, a citizen of the United States of America, and a resident of the city of St. Louis, State of Missouri, have invented certain new and useful Improvements in Methods of Casting, of which the following is a full, clear, and exact description, reference being had to the accompanying drawing, forming a part of this specification.

My invention has for its object the production of a casting in such manner as to provide therein an undercut hole into which a rivet may be driven and spread to secure it to the casting. This object is attained by my simple and inexpensive method of casting.

Figure I is a fragmentary view of a mold prepared in accordance with my method with a pattern therein.

Fig. II is a view similar to Fig. I showing a casting in the mold.

Fig. III is a cross section through a casting produced by my method, showing a rivet driven into the casting and serving to hold a third member thereto.

In carrying out my method, I make use of a sand mold and prepare the mold cavity by laying a pattern in the sand in one section of the mold and ramming the sand there-around. The pattern used is provided with a cavity the location of which corresponds to the location at which the rivet cavity is to be produced in the casting, and into this cavity in the pattern I introduce the stem of a core which terminates in an enlargement and is carried by a main body portion. The cavity in the pattern is of greater diameter throughout its length than the diameter of the enlargement at the end of the core stem, and, consequently, the stem of the core may be readily inserted into and withdrawn from said cavity.

After the core has been inserted in the pattern, as explained, I prepare the second section of the mold, ramming the sand there-in against the pattern and around the body of the core which projects above the pattern into the upper section of the mold.

When the described steps have been carried out, I lift the upper section of the mold off of the lower section, and the core, remaining seated in the upper section, withdraws or separates from the pattern embedded in the lower section. The pattern is then removed from the lower section leaving

a cavity and the upper section is replaced on to the lower section thus causing the stem of the core to be positioned in the mold cavity. Molten metal or other mobile casting material being poured into the mold fills the mold cavity and encircles the stem of the core, so that said stem with its enlarged end becomes embedded in the metal and produces an undercut cavity therein of a contour corresponding to that of the stem and its enlargement. The casting is then taken from the mold and the core is removed therefrom by destroying it through disintegration leaving the undercut cavity which is adapted to receive a rivet and cause the spreading thereof when the rivet is placed in the cavity and driven against the material at the bottom of the cavity.

The preferred procedure in practising my method is as follows:

I first prepare a pattern A in any ordinary and well known manner and provide therein a recess or pocket *a* which I locate in the pattern at a point corresponding to that at which I desire to form a rivet cavity in the casting to be molded. Said pocket extends only part way through the pattern and is preferably circular in cross section. I place the pattern on a follow-board 1 with the mouth of the pocket *a* facing said board, then place the drag 2 of a flask on said follow-board and fill it with sand which is then rammed around the pattern. The drag is next inverted to place the pattern at the top of the sand with the pocket *a* exposed.

A destructible core B (preferably of sand) is prepared and arranged in the pocket in the pattern before the cope of the flask is put in place and filled with sand. This core comprises a head 3 of tapered or other shape which provides for the head of the core being firmly held in the sand in the cope when it is rammed. The core also includes a stem 4 of less diameter than the diameter of the pocket *a* in the pattern, said stem terminating in an enlargement 5.

The core B is applied to the pattern by inserting its stem into the pocket *a*, and when the core is so applied, the terminal enlargement 5 of the core is at the bottom of said pocket.

The cope 6 of the flask is now mounted on the drag, filled with sand and rammed so that the mold, with the pattern therein, will be complete as illustrated in Fig. I. The cope is then lifted from the drag carrying

with it the core B which is then withdrawn from the pocket in the pattern. After removing the pattern from the drag, the cope, with the core still present therein, is replaced on or returned to the drag, and casting material in molten condition is poured into the mold cavity to fill it and inclose the stem of the core and its enlargement 5, as seen in Fig. II. The result is the formation 10 of a cavity in the casting having an undercut inner end of larger diameter than the portion of the cavity produced by the stem of the core. A rivet driven into such a cavity spreads at its inner end into the undercut 15 base portion of the cavity as illustrated in Fig. III, whereby the rivet is securely attached to the casting.

I claim:

1. The method of producing a casting 20 having an undercut rivet cavity therein, which consists in placing a pattern having a pocket therein in a flask drag, pouring sand into the flask drag and tamping it about the pattern, introducing into the 25 pocket a core having an enlargement at its end which enters the pocket, applying a flask cope, pouring in green sand and tamping it about the core, opening the mold, removing the pattern therefrom, closing the

mold, thereby returning the core so that the 30 enlargement at its terminal end will project into the cavity left by the removal of the pattern, and then pouring casting material in mobile condition into the cavity.

2. The method of producing a casting 35 having an undercut rivet cavity therein, which consists in placing a pattern having a pocket therein in a first mold section, pouring green sand into the first mold section and tamping it about the pattern, introducing into the pocket a core having an enlargement at its end which enters the 40 pocket and also having an enlargement toward its opposite end, forming a second mold section above the first mold section and about the exposed portion of the core, so that that part of the core will be embedded in the second mold section, removing the second mold section with the core therein, removing the pattern from the first mold section, replacing the second mold section upon the first mold section so that the portion of the core which had projected into the pocket in the pattern will project into the cavity left by the removal of the pattern and thereafter pouring casting material in mobile 45 condition into said mold cavity.

LUCAS EDEL.

Copies of this patent may be obtained for five cents each, by addressing the "Commissioner of Patents Washington, D. C."